

## UNITED STATES PATENT OFFICE

2,351,545

## MANUFACTURE OF VARNISHES

Alfred E. Rheineck and Samuel B. Crecelius,  
Louisville, Ky., assignors to Devoe & Reynolds  
Company, Inc., a corporation of New York

No Drawing. Application March 28, 1942,  
Serial No. 436,626

7 Claims. (Cl. 106—218)

The classical method of making varnishes consisted in heating together a drying oil such as linseed oil and a varnish resin such as rosin, run congo, damar, run copal or other natural resin ingredients. We have discovered that very valuable varnishes can be obtained following approximately this old procedure, provided the drying oil ingredient is saponified before being heated with the resin and then recombined with a polyhydric alcohol. Usually this will be done by neutralizing to remove the alkali, followed by subsequent esterification. When a varnish is made in this manner, the resulting product has many excellent qualities. The viscosity increases rapidly. The water resistance of the final product is definitely superior to that of comparative varnishes made from the same proportions and types of ingredients following usual procedure. There is a definite improvement in the alkali resistance, the rocker hardness is increased and these varnishes show extremely good drying qualities.

This process is particularly applicable to the drying oils having non-conjugated double bonds, and when we refer to drying oils, we are using that term quite broadly to include oils averaging at least approximately one and one-half double bonds per acid chain, so that we are including oils such as soybean oil which is sometimes classed as a semi-drying oil.

The oils may be saponified with any ordinary alkali and the saponified fatty acids may be separated from the glycerine or the glycerine may remain in the mixture, in which case it ordinarily will be removed later in the process so that it is available for subsequent esterification. If desired, previously separated fatty acids may be used. The saponification may be carried out with either a water or alcoholic solution of the alkali, but ordinarily the water solution will be employed as a matter of economy.

As regards the resin ingredient, any of the natural resins may be employed which melt at a reasonable temperature (say between 100° C. and 260° C.) and which are directly miscible with oil. If the high melting point resins which are not easily miscible with oil are to be employed, they should first be run to lower their melting point. The resins may be combined with other ingredients as in the case of ester gum or rosin modified phenolic resins, but ordinarily nothing is gained by using such products as they tend to saponify when treated with the fatty acid soaps. However, we have found that in addition to the natural resins, we may also

employ the synthetic varnish resins which are oil-soluble and fusible such as the 100% oil soluble phenolic varnish resins.

Ordinarily the resin will be pre-melted and 5 may have a small amount of some inert solvent such as mineral spirits, xylene, toluene or the equivalent added prior to the addition of soap. However, if an anhydrous soap made in an alcohol solution is employed, the premelting of the resin is not essential but is desirable to minimize 10 decomposition of the soap.

When an aqueous soap solution or wet soap 15 is used, it is gradually added to the melted resin with or without solvent at some temperature between 100° C. and 275° C. depending upon the melting point of the resin. The water will be spontaneously evaporated or distilled off with the hydrocarbon solvent, which may be separated from the water and returned. When no 20 solvent is used, open vessels can be used advantageously but in that case the wet soap must be added gradually to the melted resin due to the foaming which ensues.

After the soap has all been added to the 25 melted resin the mass is heated to a temperature of between 200° C. and 285° C., and preferably to a temperature between 240° C. and 260° C., and is maintained at the reaction temperature for a time varying from 2 to 10 hours, depending on the temperature employed. Within 30 the preferred temperature range, the desired effect ordinarily can be obtained in between 2 and 5 hours using linseed or soybean oil acid soaps. After the heating period, the soap and resin mixture is run into dilute mineral acids 35 to decompose the soap. This can be done in any way desired as is known in the art, but we find that this step can be accomplished advantageously in using a 10% excess of sulphuric acid containing about 45% of  $H_2SO_4$  by weight. After the acidification, the mass should be washed carefully, and ordinarily this will be done using 3 or 4 washes with hot water. If any glycerine remains in the soap the bulk of 45 it will be removed at this time. After elimination of the water, the acidity of the mass is determined and the acids are esterified with a polyhydric alcohol.

The amount of resin used is determined by 50 the oil length of the desired final varnish. Thus if a 25-gallon varnish is wanted, we may use 100 pounds of rosin and an amount of soap equivalent to 25 gallons of oil. This is approximately two parts of oil for one part of rosin. We have found that our process is practically

operative for various oil ranges between about 5 and 30 gallons. If one goes above 30-gallon oil length the quantity of resin present is usually insufficient properly to disperse the soaps.

The acid value of the final fatty acid-resin mixture after washing but before esterification is determined and when this figure has been obtained the amount of polyhydric alcohol required is calculated and a slight excess over the stoichiometric quantity is ordinarily employed. Various polyhydric alcohols may be employed such as glycerol, erythritol, pentaerythritol, mannitol, sorbitol and inositol or mixtures of these. Esterification is brought about by heating the mixture of alcohol and acids by any well-known manner as is known in the art. Ordinarily heating will be continued at temperatures between 200° C. and 300° C. until the acid value reaches 10 to 15 which requires from 6 to 8 hours.

During the final portion of the esterification reaction, the temperature is preferably raised somewhat, say to 280° to 290° C., in order to body the product. In our practice, we consider that the final step is completed when samples thinned with an equal weight of mineral spirits have a viscosity between E and G on the Gardner-Holdt scale. This final bodying step may take about 2 hours but as pointed out, the bodying and esterification may be carried out simultaneously.

We have also found that the steps of neutralization and esterification can be avoided by using a polyhalogenated polyhydric alcohol which will react directly with the fatty acid soaps. For example, if a mixture containing approximately 2 mols of fatty acid soap for each mol of a natural resin is treated with dichlorohydrin, a reaction will take place with the precipitation of the alkali salt, and the resin acids can be esterified with the residual hydroxyl groups of the dichlorohydrin. Where larger amounts of resin are present, mixtures of monochlorohydrin and dichlorohydrin can be employed. On the other hand, where a varnish is being prepared of a relatively high oil length, a small amount of the soap may be neutralized, as for example with a bisulphate or monophosphate or even with small quantities of an acid such as sulphuric or hydrochloric acid. In such case the released fatty acids can react with the hydroxyls of the halogenated polyhydric alcohol or with other polyhydric alcohol which may be added. Obviously in addition to the halogenated glycerides, other halogenated polyhydric alcohols may be employed.

This process is particularly useful with any oil which contains appreciable amount of fatty acid groups having at least two double bonds in the isolated position, that is, non-conjugated. Such oil may include, for example, linseed oil, fish oil, soybean oil, perilla oil or their equivalents. The process may also be employed with oils having some or all of their double bonds in conjugated positions as for example with dehydrated castor oil. In such case the benefits of our process are not always so apparent.

Our process can readily be understood from the following illustrative examples which show some preferred forms of carrying out the same:

#### Example I

500 parts of WG rosin was melted and heated at a temperature of between 200° C. and 240° C. in an open kettle. 5085 parts of a linseed soap

solution equivalent to 1000 parts of linseed oil was added slowly over a period of 2 hours while the mixture was stirred gently. The rate of soap addition was determined by the rate of foaming.

5 After the soap solution was added, the rosin soap mixture was heated at 260° C. for 3 hours. The rosin fatty acid mixture was recovered by treating the rosin soap mixture with a slight excess of 45% sulphuric acid. The freed acids were thoroughly washed with water and dried. The final acid value was 169.

15 300 parts of these acids was mixed with 29 parts of glycerol and the mixture was heated for 3 hours at a temperature of between 180° C. and 200° C. The temperature was then raised to 260° C. and held for 12 hours while carbon dioxide was passed through the mixture. At the end of that time the mixture was thinned with mineral spirits to yield a varnish containing 55% solids and was treated with .75% Pb and .06% Co as driers. The varnish had a viscosity of D on the Gardner-Holdt scale and an acid value of 6.

#### Example II

25 600 parts of linseed fatty acids was heated to about 100° C. and 117 parts of sodium methoxide was gradually added. The resulting soapy mass was heated to about 110°-120° C. and cooled. 300 parts of 99% abietic acid was melted at a temperature of between 110° and 150° and the spongy soap was added. The mixture was then gradually heated with stirring to a temperature of 240° C. and held for 5 hours. The soap was decomposed with 45% sulphuric acid and the final acid value was 186.

40 790 parts of these acids was mixed with 84 parts of glycerol and this mixture was heated with stirring for 6 hours at a temperature of between 230° and 240° C. with passage of carbon dioxide. The resulting product showed a viscosity of Z-6 on the Gardner-Holdt scale and an acid value of 7.5. For the purpose of comparison 600 parts of linseed fatty acids was heated with 300 parts of 99% abietic acid and esterified with glycerol. The resulting product had a viscosity of M on the Gardner-Holdt scale and an acid value of 11.5.

#### Example III

250 parts of run East India resin was heated to a temperature of between 200° and 240° C. in an open kettle and linseed soap paste equivalent to 500 parts of linseed oil was gradually added and the resulting mixture was heated to 260° C. for 3 hours. After neutralization with sulphuric acid and thorough washing the final acid value of the mixture was 139. In order to prepare a 25-gallon varnish from these acids they were acidified with 20 parts of glycerol. The resulting solids were thinned with mineral spirits to 50% solids and driers added as before. The final varnish had a viscosity of L on the Gardner-Holdt scale and an acid value of 4.7.

#### Example IV

400 parts of rosin was melted as in Example I and as before was treated with linseed soap paste equivalent to 400 parts of linseed oil. After following out the procedure outlined in Example I through the point of neutralization, the mixture showed an acid value of 145. 275 parts of these acids was esterified with 23 parts of glycerol to produce a 1½ gallon varnish. After esterification was completed the mass was thinned with mineral spirits to 50% solids and treated with

driers as before. The resulting varnish showed a viscosity of between E and F on the Gardner-Holdt scale and an acid value of 1.8.

It is understood that these examples are given only by way of illustration and that the same may be modified in many particulars without departing from the spirit of our invention.

What we claim is:

1. In the process of making varnishes the steps which comprise heating together for at least about two hours soaps of drying oil fatty acids having non-conjugated double bonds and an oil soluble varnish resin in proportions to give a varnish length of between 5 and 30 gallons and at a temperature of between 200° C. and 285° C., and subsequently forming a polyhydric alcohol ester of the fatty acids represented in the soap, in the presence of such resin.

2. A process as specified in claim 1 in which the resin is a natural varnish resin and the fatty acids are liberated with acid and subsequently the fatty acids and natural resin acids are esterified with a polyhydric alcohol.

3. A process as specified in claim 1 in which the polyhydric alcohol is halogenated and the

halogenated alcohol is caused to react directly with the soaps.

4. A process as specified in claim 1 in which the temperature is in excess of 240° C.

5. In the process of making varnishes, the steps which comprise adding water wet soap of drying oil fatty acids having non-conjugated double bonds to melted natural varnish resin, heating the resulting mixture to a temperature of between 200° C. and 285° C. for from 2 to 10 hours, adding acid to release the fatty acids, washing and esterifying the fatty acids and resin acids with a polyhydric alcohol.

10 6. A process as specified in claim 5 in which the temperature is between 240° C. and 260° C.

7. In the process of making varnishes from varnish resins and drying oils having non-conjugated bonds, the steps of forming a soap of the fatty acids of such drying oil and heating such soap with an oil-soluble varnish resin for at least 15 two hours at a temperature of between 200° C. and 285° C., the resin being present in proportion to give a varnish length of between 5 and 30 gallons.

ALFRED E. RHEINECK.  
SAMUEL B. CRECELIUS.